

1

3,687,605

**STABILIZATION OF WOOL THROUGH TREATMENT WITH A REDUCING AGENT AND A POLYMER OR POLYMER FORMING MATERIALS**  
Larry B. Farmer, Spartanburg, S.C., assignor to Deering Milliken Research Corporation, Spartanburg, S.C.  
No Drawing. Filed Mar. 14, 1966, Ser. No. 533,844  
Int. Cl. D06m 3/08, 3/10, 15/30  
U.S. Cl. 8—127.6

6 Claims

## ABSTRACT OF THE DISCLOSURE

A two step durable setting in the desired configuration of textile materials containing keratinous fibers comprising (1) an external stabilization and (2) an internal stabilization. The external stabilization involves polymer formation through treatment with a polyisocyanate and an active hydrogen containing polymer. The internal stabilization involves treatment with a reducing agent.

This invention relates to a textile fabric which contains keratinous fibers and which has a propensity to conform durably to a preselected configuration, and more specifically, to wool fabrics having creases which are durable to laundering and dry cleaning operations.

Garments prepared from cellulosic fabrics having creases set therein which are durable to laundering have recently found wide acceptance in the textile industry. Cellulosic garments of the aforementioned types and the methods for their preparation are set forth in U.S. Patent No. 2,974,432. A satisfactory process for the preparation of durable creases in wool fabrics which will withstand home laundering operations, however, has not heretofore been found.

Garments made from wool fabrics have been sprayed with reducing agent solutions and pressed on a steam press in an attempt to produce durable creases in the garments. The creases as produced are quite durable to mere wetting but will not withstand a combination of wetting and agitation, such as occurs in a washing machine.

It has now been discovered that configurations which will withstand washing can be produced in wool garments by subjecting the fabric to an external stabilizing operation, treating the externally stabilized fabric with a reducing agent, maintaining the reducing agent treated fabric in a desired configuration while reforming the split linkages of the keratinous fibers.

The preferred process for splitting internal linkages of keratinous fibers is treatment with a reducing agent. Preferred among the linkage reforming processes are steam and heat processes. The preselected configurations which are contemplated include any shape desired in the fabrics or garments made from such fabrics, e.g., pleats, creases, texturing effects, such as pebble textures, and the like.

The external setting of the keratinous fiber is accomplished by means of a polymeric chemical reagent. Typical examples of such setting processes are additive type shrinkproofing processes wherein polymeric reagents are added to keratinous fabrics. These reagents preferably react with the keratinous component for improved washability characteristics. It should be understood, however, that the external stabilization of the keratinous fiber may also be accomplished by means of coating the fibers with a non-reactive polymeric coating composition so as to secure the fibers in the desired configuration by means of the mechanical forces exerted by the coating, e.g., according to the Wurlan process developed at the Western Regional Laboratories of the United States Department of

2

Agriculture. While the preferred external setting medium is a medium of the type which produces new chemical bonds by reacting with a keratin fiber, the only prerequisite for this type of reagent is that at least some of the new chemical bonds be formed on the surface of the keratinous fiber, that is to say chemical bonds may be formed internally and externally, but at least some bonds must be formed on the surface of the fiber. Systems which have been found to be especially suitable for the external

5 stabilization of this invention are interfacial polymerization systems such as those involving the formation of poly(hexamethylene sebacate) through interfacial polymerization techniques, treatments with reactive terpolymers based on vinyl type monomers, treatments with poly-10 epoxide-polyamine compositions, treatments with reactive polyurethanes and treatments with emulsions of certain acrylic esters such as, for instance, polymethylmethacrylate, polyethylmethacrylate, polypropylmethacrylate and polybutylmethacrylate.

15 20 The use of polymeric external stabilizing agents provides many advantages over techniques involving the use of monomeric oxidizing agents such as sodium chlorite and various permanganate salts. Polymeric compounds not only provide a higher level of stability to washing in fabrics so treated, but also provide a higher level of finish 25 stability as well as flat drying properties than is possible with monomeric type treating agents. In other words, when a wool fabric is first treated with a monomeric shrinkproofing agent and then durably set with reducing 30 agent solutions, the results, if anything, are less than additive. The fabric, during washing, tends to shrink slightly more than if no reducing agent treatment had been employed and the flat drying properties and finish 35 are not satisfactory. On the other hand, when a polymeric shrinkproofing agent is utilized in combination with the reducing agent treatment, a synergistic effect on crease retention, flat drying properties and finish stability is attained in that these properties are far superior to the same properties measured on the fabric after either treatment 40 separately.

45 The most preferred external stabilizing agents for purposes of the invention are isocyanate reaction products. These reaction products, in combination with the internal stabilizing treatment, provide greatly improved washability characteristics. For example, garments made from fabrics treated with these products accept creases quite readily and retain these creases after washing and tumble drying to a much greater extent when compared with other externally stabilized fabrics, although these 50 latter products are entirely satisfactory.

55 Among the isocyanate reaction products which may be employed are isocyanate reaction products selected from two general categories, the first of which is a urethane prepared from a polyfunctional isocyanate and a polymeric polyhydroxy compound and the second of which is the reaction product of a polyfunctional isocyanate and polymeric polyfunctional compound selected from the group consisting of polyesters, polyamides, poly-epoxides and reaction products of phenol and alkanol oxides, form-60 aldehyde resins, hydrogenation products of olefin-carbon monoxide copolymers and polyepihalohydrins. It should be understood that the isocyanate reaction products may be applied to the fabric as a single solution in pre-polymer form or in "one-shot" applications forming the isocyanate reaction product on the fabric in situ.

65 70 Regardless of the system utilized, it is preferred that the ratio of isocyanate to active hydrogen compound be at least about 0.4, but most preferably, greater than 1.0, e.g., from 1.01 to about 2.0, preferably 1.05 to 1.6. Systems containing an excess of isocyanate are much more highly reactive with keratin fibers, so that stabilization is provided to the desired level, permitting washing with

little or no degradation of the hand, or feel, of the fabric. Surprisingly, configurations imparted to such fabrics by subsequent reducing agent treatments are durable to washing even at low levels of polymer, e.g., as little as 1%, but preferably between 3 and 10%, although amounts on the order of 15-25% produce excellent results, even though producing stiffening effect on fabric so treated.

By "pre-polymer" herein is meant the reaction product of the polyfunctional isocyanate and the preselected second polymeric compound carried to an extent below which a gel is produced which is insoluble in one of the organic solvents for each of the two reaction components and particularly the chlorinated hydrocarbons. When the pre-polymer is prepared from an excess of isocyanate as preferred, the resulting product is believed to be an isocyanate-terminated polyurethane, which is highly reactive with keratin fibers.

The term "one-shot" as employed herein is meant to define a process wherein the isocyanate and active hydrogen compound are applied to the substrate material directly from solution. The desired polymer is then formed *in situ* on the fabric. In general, the degree of polymerization of the resulting polymer exceeds that of the pre-polymer.

Among the suitable isocyanates that may be used in accordance with this invention are included aryl diisocyanates such as 2,4-tolylene diisocyanate, 2,6-tolylene diisocyanate, 4,4'-diphenylmethane diisocyanate, p-phenylene diisocyanate, 1,5-naphthylene diisocyanate, m-phenylene diisocyanate, diphenyl-4,4'-diisocyanate, azobenzene-4,4'-diisocyanate, diphenylsulphone-4,4'-diisocyanate, 1-isopropylbenzene-3, 5-diisocyanate, 1-methyl-phenylene-2,4-diisocyanate, naphthylene-1,4-diisocyanate, diphenyl-4,4'-diisothiocyanate and diisocyanate, benzene-1, 2,4-triisothiocyanate, 5-nitro-1,3-phenylene diisocyanate, xylylene-1,4-diisocyanate, xylylene-1,3-diisocyanate, 4,4'-diphenylene-methane diisocyanate, 4,4'-diphenylene-propane diisocyanate and xylylene-1,4-diisothiocyanate and the like; aliphatic diisocyanates, such as dicyclohexamethane-4,4'-diisocyanate and the like; alkylene diisocyanates such as tetramethylene diisocyanate, hexamethylene diisocyanate and the like, as well as mixtures thereof and including the equivalent isothiocyanates. Of these compounds, the aryl diisocyanates are preferred because of their solubility and availability.

Additional isocyanates include polymethylene diisocyanates and diisothiocyanates, such as ethylene diisocyanate, dimethylene diisocyanate, dodecamethylene diisocyanate, hexamethylene diisocyanate, tetramethylene diisocyanate, pentamethylene diisocyanate, and the corresponding diisothiocyanates; alkylene diisocyanates and diisothiocyanates such as propylene-1,2-diisocyanate, 2,3-dimethyltetra-methylene diisocyanate and diisothiocyanate, butylene-1,2-diisocyanate, butylene-1,3-diisothiocyanate, and butylene-1,3-diisocyanate; alkylidene diisocyanates and diisothiocyanates such as ethylidene diisocyanate



and heptylidene diisothiocyanate



cycloalkylene diisocyanates and diisothiocyanates such as 1,4-diisocyanatocyclohexane, cyclopentylene-1,3-diisocyanate, and cyclohexylene-1,2-diisothiocyanate; aromatic polyisocyanates and polyisothiocyanates such as aliphatic-aromatic diisocyanates and diisothiocyanates such as phenylethylene diisocyanate ( $C_6H_5CH(NCO)CH_2NCO$ ); diisocyanates and diisothiocyanates containing heteroatoms such as  $SCNCH_2OCH_2NSC$ ,



and  $SCN(CH_2)_3-S-(CH_2)_3NSC$ ; 1,2,3,4-tetraisocyanatobutane, butane-1,2,2-triisocyanate, tolylene-2,4,6-triisocyanate, tolylene-2,3,4-triisocyanate, benzene-1,3,5-tri-

isocyanate, benzene-1,2,3-triisocyanate, 1-isocyanato-4-isothiocyanatohexane, and 2-chloro-1,3-diisocyanatopropane.

The preferred diisocyanates, diisothiocyanates and mixed isocyanate-isothiocyanates have the general formula  $ZCN-R-NCZ$  in which R is a divalent hydrocarbon radical, preferably aryl, and Z is a chalcogen of atomic weight less than 33. For availability, tolylene 2,4-diisocyanate is preferred.

- 10 By "polymeric polyhydroxy compound" is meant a linear long-chain polymer having terminal hydroxyl groups including branched, polyfunctional polymeric hydroxy compounds as set forth below. Among the suitable polymeric polyhydroxy compounds, there are included 15 polyether polyols such as polyalkyleneether glycols, and polyalkylene-aryleneether-thioether glycols and polyalkyleneether triols. Polyalkyleneether glycols and triols are preferred. Mixtures of these polyols may be used when desired.
- 20 The polyalkyleneether glycols may be represented by the formula  $HO(RO)_nH$ , wherein R is an alkylene radical which need not necessarily be the same in each instance and n is an integer. Representative glycols include polyethyleneether glycol, polypropyleneether glycol, polytrimethyleneether glycol, polytetramethylene ether glycol, polypentamethyleneether glycol, polydecamethyleneether glycol, polytetramethylene formal glycol and poly-1,2-dimethylethyleneether glycol. Mixtures of two or more polyalkyleneether glycols may be employed if desired.
- 25 Representative polyalkyleneether triols are made by reacting one or more alkylene oxides with one or more low molecular weight aliphatic triols. The alkylene oxides most commonly used have molecular weights between about 44 and 250. Examples include: ethylene oxide; propylene oxide; butylene oxide; 1,2-epoxybutane; 1,2-epoxyhexane; 1,2-epoxyoctane; 1,2-epoxyhexadecane; 2,3-epoxybutane; 3,4-epoxyhexane; 1,2-epoxy-5-hexene; and 1,2-epoxy-3-butane, and the like. Ethylene, propylene, and butylene oxides are preferred. In addition to mixtures of these oxides, 30 minor proportions of alkylene oxides having cyclic substituents may be present, such as styrene oxide, cyclohexene oxide, 1,2-epoxy-2-cyclohexylpropane, and a methyl styrene oxide. The aliphatic triols most commonly used have molecular weights between about 92 and 250. Examples include glycerol, 1,2,6-hexanetriol; 1,1,1-trimethylolpropane; 1,1,1-trimethylolethane; 2,4-dimethylol-2-methylol-pentanediol-1,5 and the trimethylether of sorbitol.

- 35 Representative examples of the polyalkyleneether triols include: polypropyleneether triol (M.W. 700) made by reacting 608 parts of 1,2-propyleneoxide with 92 parts of glycerine; polypropyleneether triol (M.W. 1535) made by reacting 1401 parts of 1,2-propyleneoxide with 134 parts of trimethylolpropane; polypropyleneether triol (M.W. 2500) made by reacting 2366 parts of 1,2-propyleneoxide with 134 parts of 1,2,6-hexanetriol; and polypropyleneether triol (M.W. 6000) made by reacting 5866 parts of 1,2-propyleneoxide with 134 parts of 1,2,6-hexanetriol.

- 40 Additional suitable polytriols include polyoxypropylene triols, polyoxybutylene triols, Union Carbide's Niax triols LG56, LG42, LG112 and the like; Jefferson Chemical's Triol G-4000 and the like; Actol 32-160 from National Aniline and the like.

- 45 The polyalkylene-aryleneether glycols are similar to the polyalkyleneether glycols except that some arylene radicals are present. Representative arylene radicals include phenylene, naphthalene and anthracene radicals which may be substituted with various substituents, such as alkyl groups. In general, in these glycols there should be at least one alkyleneether radical having a molecular weight of about 500 for each arylene radical which is present.

- 50 The polyalkylene-aryleneether-thioether glycols and the polyalkylene-aryleneether glycols are similar to the above-described polyether glycols, except that some of the ether-oxygen atoms are replaced by sulfur atoms. These glycols

may be conveniently prepared by condensing together various glycols, such as thiodiglycol, in the presence of a catalyst, such as p-toluene-sulfonic acid.

By "polymeric polyfunctional compound" is meant a long-chain polymer of the types described containing at least two groups having at least one active hydrogen atom as determined by the Zerewitinoff method. In the process of this invention, there may be utilized such compounds as polyesters, polyamides, polyepoxides, reaction products of phenols and alkylene oxides, formaldehyde resins, hydrogenation products of olefine-carbon monoxide copolymers, and polyepihalohydrins.

The polyesters suitable for use in accordance with this invention are well known and are generally prepared by conducting a condensation reaction between an excess of a monomeric or polymeric polyhydroxy compound and a polyacid or by esterifying a hydroxy substituted acid and a polyhydroxy alcohol.

Among the suitable acids there are included the alkane dibasic acids, alkene dibasic acids, cycloalkene dibasic acids, cycloalkane dibasic acids, aryl dibasic acids, or any of the foregoing types wherein the hydrocarbon radical is substituted with an alkyl, alkenyl, cycloalkyl, cycloalkenyl or aryl radical.

Representative dibasic carboxylic acids which can be employed for reaction with polyols in preparation of polyesters for use in accordance with this invention include the following: succinic; monomethyl succinic; glutaric; adipic; pimelic; suberic; azelaic; sebacic; brassylic; thapsic; 6-oxoundecanedioic; octadecanedioic acid; 8-octadecenedioic acid; ricinoleic acid; 6,8-octadecadienedioic acid; malic; and the like. Other acids include: unsaturated acids such as maleic, fumaric, glutaconic, and itaconic; the cycloalkane dicarboxylic acids such as cyclopentane-1,2-dicarboxylic and cyclopentane-1,3-dicarboxylic; aromatic dicarboxylic acids such as phthalic, isophthalic, terephthalic, naphthalene - 1,2 - dicarboxylic, naphthalene - 1,3 - dicarboxylic, naphthalene-1,4-dicarboxylic, naphthalene-1,5-dicarboxylic, naphthalene-1,8-dicarboxylic, diphenyl-2,2'-dicarboxylic, diphenyl-4,4'-dicarboxylic and diphenyl-2,4'-dicarboxylic; and aliphatic-aromatic dicarboxylic acids such as 2,6 - dimethylbenzene-1,4-dicarboxylic acid, and 4,5-dimethylbenzene-1,2-dicarboxylic acid; and the like. Natural products which are particularly useful include castor oil, which comprises a glyceride of ricinoleic acid, and rincinoleyl alcohol, and mixtures thereof.

Representative monomeric polyols for reaction with the above acids for the production of polyesters for use in accordance with this invention include the polyalkylene-ether glycols represented by the formula  $\text{HO}(\text{RO})_n\text{H}$ , wherein R is an alkylene radical which need not necessarily be the same in each instance and n is an integer. Representative glycols include polyethylenether glycol, polypropyleneether glycol, polytrimethyleneether glycol, polytetramethyleneether glycol, polypentamethyleneether glycol, polydecamethyleneether glycol, polytetramethyleneformal glycol and poly-1,2-dimethylethyleneether glycol. Mixtures of two or more polyalkyleneether glycols may be employed if desired.

Representative polyalkyleneether triols are made by reacting one or more alkylene oxides with one or more low molecular weight aliphatic triols. The alkylene oxides most commonly used have molecular weights between about 44 and 250. Examples include: ethylene oxide; propylene oxide; butylene oxide; 1,2-epoxybutane; 1,2-epoxyhexane; 1,2-epoxyoctane; 1,2-epoxyhexadecane; 2,3-epoxybutane; 3,4-epoxyhexane; 1,2-epoxy-5-hexene; and 1,2-epoxy-3-butane, and the like. Ethylene, propylene, and butylene oxides are preferred. In addition to mixtures of these oxides, minor proportions of alkylene oxides having cyclic substituents may be present, such as styrene oxide, cyclohexene oxide, 1,2-epoxy-2-cyclohexylpropane, and a-methyl styrene oxide. The aliphatic triols most commonly used have molecular weights between about 92 and 250. Examples include glycerol; 1,2,6-hexanetriol; 1,1,1-tri-

methylolpropane; 1,1,1-trimethylolethane; 2,4-dimethylol-2-methylol-pentanediol-1,5 and the trimethylether of sorbitol.

Representative examples of the polyalkyleneether triols include: polypropyleneether triol (M.W. 700) made by reacting 608 parts of 1,2-propyleneoxide with 92 parts of glycerine; polypropyleneether triol (M.W. 1535) made by reacting 1401 parts of 1,2-propyleneoxide with 134 parts of trimethylopropane; polypropyleneether triol (M.W. 2500) made by reacting 2366 parts of 1,2-propyleneoxide with 134 parts of 1,2,6-hexanetriol; and polypropyleneether triol (M.W. 6000) made by reacting 5866 parts of 1,2 - propyleneoxide with 134 parts of 1,2,6-hexanetriol.

Additional suitable polytriols include polyoxypropylene triols, polyoxybutylene triols, Union Carbide's Niax triols LG56, LG42, LG112 and the like; Jefferson Chemical's Triol G-4000 and the like; Actol 32-160 from National Aniline and the like.

The polyalkylene-aryleneether glycols are similar to the polyalkyleneether glycols except that some arylene radicals are present. Representative arylene radicals include phenylene, naphthalene and anthracene radicals which may be substituted with various substituents, such as alkyl groups. In general, in these glycols there should be at least one alkyleneether radical having a molecular weight of about 500 for each arylene radical which is present.

The polyalkyleneether-thioether glycols and the polyalkylene-aryleneether glycols are similar to the above described polyether glycols, except that some of the ether-oxygen atoms are replaced by sulfur atoms. This glycols may be conveniently prepared by condensing together various glycols, such as thiodiglycol, in the presence of a catalyst, such as p-toluene-sulfonic acid.

Additional polyesters include those obtained by reacting one or more of the above acids with a mixture of polyhydric alcohols comprising (1) polyhydric alcohols of the general formula:



wherein alkylene means a divalent saturated aliphatic radical having at least 2 carbon atoms, preferably not more than 5 carbon atoms, x, y and z are whole numbers and the sum of x, y and z is from 3 to 10, preferably from 3 to 6, at least two of the  $-(\text{alkylene-O})_{xyz}\text{H}$  groups contain primary alcoholic hydroxyl groups and R is a large alkyl group containing from 10 to 25 carbon atoms, and (2) polyhydric alcohols containing only carbon, hydrogen and oxygen, and the polyhydric alcohols from (1) and (2) are employed in such proportions that from 1 to 15 alcoholic OH groups are contributed by (1) for every 10 alcoholic OH groups contributed by (2).

The polyepoxides used in accordance with the invention are organic compounds having at least two epoxy groups per molecule and may be saturated or unsaturated, aliphatic, cycloaliphatic, aromatic or heterocyclic and may be substituted with non-interfering substituents such as hydroxyl groups, ether radicals, and the like. Polyepoxides containing ether groups, generally designated as polyepoxide polyethers, may be prepared as well known in the art by reacting a polyol with a halogen-containing epoxide employing at least 2 moles of the halogen-containing epoxide per mole of polyol. Thus, for example, epichlorohydrin may be reacted with a polyhydric phenol in an alkaline medium. In another technique the halogen-containing epoxide is reacted with a polyhydric alcohol in the presence of an acid-acting catalyst such as hydrofluoric acid or boron trifluoride and the product is then reacted with an alkaline compound to effect a dehydrohalogenation. A preferred example of the halogen-containing epoxide is epichlorohydrin; others are epibromo-

hydrin, epiodohydrin, 3-chloro-1,2-epoxybutane, 3-bromo-1,2-epoxyhexane, and 3-chloro-1,2-epoxy-octane. Illustrative examples of polyepoxide polyethers are as follows:

1,4 - bis(2,3 - epoxypropoxy)benzene; 1,3 - bis(2,3-epoxypropoxy - benzene) 4,4'-bis(2,3-epoxypropoxy)di-phenyl ether; 1,8 - bis(2,3 - epoxypropoxy)octane; 1,4-bis(2,3 - epoxypropoxy)cyclohexane; 4,4' - bis(2 - hydroxy - 2,4 - epoxybutoxy) diphenyl dimethylmethane; 1,3 - bis(4,5 - epoxypentoxy) - 5 - chlorobenzene; 1,4-bis(3,4 - epoxybutoxy) - 2 - chlorohexane; diglycidyl thioether; diglycidyl ether; ethylene glycol diglycidyl ether; propylene glycol diglycidyl ether; diethylene glycol diglycidyl ether; resorcinol diglycidyl ether; 1,2,3,4-tetrakis (2 - hydroxy - 3,4 - epoxybutoxy)butane; 2,2-bis(2,3 - epoxypropoxyphenyl)propane; glycerol triglycidyl ether; mannitol tetraglycidyl ether; pentaerythritol tetraglycidyl ether; sorbitol tetraglycidyl ether; glycerol di-glycidyl ether; etc. It is evident that the polyepoxide polyethers may or may not contain hydroxy groups, depending primarily on the proportions of halogen-containing epoxide and polyol employed. Polyepoxide polyethers containing polyhydroxyl groups may also be prepared by reacting, in known manner, a polyhydric alcohol or polyhydric phenol with a polyepoxide in an alkaline medium. Illustrative examples are the reaction product of glycerol and diglycidyl ether, the reaction product of sorbitol and bis(2,3-epoxy-2-methylpropyl)ether, the reaction product of pentaerythritol and 1,2,3,5-diepoxy pentane, the reaction product of 2,2-bis(parahydroxyphenyl)propane and bis(2,3 - epoxy - 2 - methylpropyl)ether, the reaction product of resorcinol and diglycidyl ether, the reaction product of catechol and diglycidyl ether, and the reaction product of 1,4-dihydroxy-cyclohexane and diglycidyl ether.

Polyepoxides which do not contain ether groups may be employed as for example 1,2,5,6-diepoxyhexane; butadiene dioxide (that is, 1,2,3,4-diepoxybutane); isoprene dioxide; limonene dioxide.

For use in accordance with the invention, I prefer the polyepoxides which contain ether groups, that is, polyepoxide polyethers. More particularly I prefer to use the polyepoxide polyethers of the class of glycidyl polyethers of polyhydric alcohols or glycidyl polyethers of polyhydric phenols. These compounds may be considered as being derived from a polyhydric alcohol or polyhydric phenol by etherification with at least two glycidyl groups—



The alcohol or phenol moiety may be completely etherified or may contain residual hydroxy groups. Typical examples of compounds in this category are the glycidyl polyethers of glycerol, glycol, diethylene glycol, 2,2-bis (parahydroxyphenyl)propane, or any of the other polyols listed hereinabove as useful for reaction with halogen-containing epoxides. Many of the specific glycidyl polyethers derived from such polyols are set forth hereinabove. Particularly preferred among the glycidyl polyethers are those derived from 2,2-bis(parahydroxyphenyl)propane and those derived from glycerol. The compounds derived from the first-named of these polyols have the structure—



wherein  $n$  varies between zero and about 10, corresponding to a molecular weight about from 350 to 8,000. Of this class of polyepoxides it is preferred to employ those compounds wherein  $n$  has a low value, i.e., less than 5, most preferably where  $n$  is zero.

In commerce, the polyepoxide polyethers are conventionally termed as epoxy resins even though the com-

pounds are not technically resins in the state in which they are sold and employed because they are of relatively low molecular weight and thus do not have resinous properties as such. It is only when the compounds are cured that true resins are formed. Thus it will be found that manufacturer's catalogs conventionally list as epoxy resins such relatively low-molecular weight products as the diglycidyl ether of 2,2-bis(parahydroxyphenyl)propane, the diglycidyl ether of glycerol, and similar polyepoxide polyethers having molecular weights substantially less than 1,000.

It is within the purview of the invention to employ mixtures of different polyepoxides. Indeed, it has been found that especially desirable results are attained by employing mixtures of two commercially available polyepoxides, one being essentially a diglycidyl ether of glycerol, the other being essentially a diglycidyl ether of 2,2 - bis(parahydroxyphenyl)propane. Particularly preferred to attain such result are mixtures containing more than 1 and less than 10 parts by weight of the glycerol diglycidyl ether per part by weight of the diglycidyl ether of 2,2-bis(parahydroxyphenyl)propane.

The polyamides used in accordance with the invention are those derived from polyamines and polybasic acids.

25 Methods of preparing these polyamides by condensation of polyamines and polycarboxylic acids are well known in the art. One may prepare polyamides containing free amino groups or free carboxylic acid groups or both free amino and free carboxylic acid groups. The polyamides 30 may be derived from such polyamines as ethylene diamine, diethylene triamine, triethylene tetramine, tetra-ethylene pentamine, 1,4-diaminobutane, 1,3-diaminobutane, hexamethylene diamine, 3-(N-isopropylamino)propylamine, 3,3'-imino-bispropylamine, and the like. Typical polycarboxylic acids which may be condensed with the polyamines to form polyamides are glutaric acid, adipic acid, pimelic acid, suberic acid, acellic acid, sebacic acid, isophthalic acid, terephthalic acid, betamethyl adipic acid, 1,2-cyclohexane dicarboxylic acid, malonic acid, polymerized fatty acids, and the like. Depending on the amine and acid constituents and the conditions of condensation, the polyamides may have molecular weights varying about from 1,000 to 10,000 and melting points about from 20-200° C. Particularly preferred for the 45 purpose of this invention are the polyamides derived from aliphatic polyamines and polymeric fatty acids. Such products are disclosed for example by Cowan et al., Pat. No. 2,450,940. Typical of these polyamides are those made by condensing ethylene diamine or diethylene 50 triamine with polymeric fatty acids produced from the polymerization of drying or semi-drying oils, or the free acids, or simple aliphatic alcohol esters of such acids. The polymeric fatty acids may typically be derived from such oils as soybean, linseed, tung, perilla, oiticica, cottonseed, corn, tall, sunflower, safflower, and the like. As well known in the art, in the polymerization the unsaturated fatty acids combine to produce a mixture of dibasic and higher polymeric acids. Usually the mixture contains a preponderant proportion of dimeric acids with lesser amounts of trimeric and higher polymeric acids, and some residual monomeric acid. Particularly preferred are the polyamides of low melting point (about 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 88

ized fatty acids, like the polyepoxides, are often referred to in the trade as resins even though not actually resins in the state in which they are sold and applied. Particularly good results are obtained in the use of low molecular weight, non-fiber forming polyamides sold under the trade name of Versamids.

Any suitable condensation product of a phenol and an alkylene oxide may be used such as, for example, the condensation product of cresol or 4,4'-isopropylidenediphenol with one of the aforementioned alkylene oxides.

Any suitable hydrogenation product of olefin-carbon monoxide copolymers may be used such as, for example, the hydrogenation product of an ethylene-propylene-carbon monoxide copolymer and others disclosed in U.S. Patent 2,839,478, issued to Wilms et al., June 17, 1958, and U.S. Patent 2,495,292, issued to Scott, Jan. 24, 1950.

In the process of this invention, it is preferred to react the polyfunctional isocyanate and polymeric polyfunctional compound or polyfunctional isocyanate and polymeric polyhydroxy compound as the case may be with or without a coreactant and unblocked or blocked in a "one-shot" procedure with the keratinous fibers in the presence of a catalyst. Any of the well-known catalysts for the reaction of active hydrogen atoms with isocyanates may be used. Of these catalysts which are used in the production of polyurethanes, organo-tin or organo-zinc compounds are preferred. Particularly preferred are either stannous octoate or zinc naphthenate.

The various isocyanate reaction product systems described above preferably are applied to the keratinous fiber containing fabric in the form of a solution, the solution employing a non-reactive solvent although aqueous emulsions may be utilized if desired. By "non-reactive" as used herein is meant a solvent in which reactivity between the isocyanate and active-hydrogen containing components of the solvent mixture even in the presence of catalyst is substantially inhibited. Small amounts of reactive solvents may be present provided the amount present is sufficiently low as not to precipitate a substantial amount of the components with which it is reacted. In other words, sufficient components remain reactive with the keratin fibers to provide adequate inhibition of shrinkage and/or settability in the fabric or other structure being treated.

Suitable organic solvents include halogenated hydrocarbons such as trichloroethylene, methylene chloride, perchloroethylene, ethylene dichloride, chloroform and the like, aromatic solvents such as toluene, xylene, benzene, mixed aromatics, such as the Solvesso types and the like, n-butyl acetate, n-butyl ether, n-butyl phosphate, p-dioxane, ethyl oxalate, methyl isobutyl ketone, pyridine, quinoline, N,N-dimethylformamide, N,N-dimethylacetamide, dimethylsulfoxide, 2,2,4-trimethyl-pentane and the like. Mixtures of solvents may be used.

The internal setting of the keratinous fibers is preferably accomplished by means of a reducing agent. Such compounds are well-known in the art and have the ability to rupture polymeric linkages, within the structure of keratin. These ruptured linkages, specifically the disulfide linkages, may be at least partially reformed while holding the fiber in a desired configuration, thereby setting this configuration durably in the fiber. The reaction which appears to take place in setting the keratinous fibers in the new shape is reformation of the cystine linkage and reformation of hydrogen bonds and/or hydrophobic bonds of the keratinous fibers, the bonds and linkages having previously been split by contact with the reducing agent. The cystine linkages are split and reunited to form at least some of the disulfide bonds. While the keratinous fibers remain substantially unchanged chemically by the reduction and oxidation operations, some relocation of the cystine linkages apparently takes place along with some changes in hydrogen and/or hydrophobic bonding. These changes in location of cystine linkages and changes in hydrogen and hydrophobic bonding produce a re-

formed fiber. The reformation of the fiber gives the individual keratinous fibers of this invention their internal setting which results in a fabric which has stabilization to dimensional and finish changes.

5 Among the suitable reducing agents, there are included lower alkanolamine sulfites, such as monoethanolamine sulfite and isopropanolamine sulfites, and others containing up to about 8 carbon atoms in the alkyl chain, such as n-propanolamine sulfite, n-butanolamine sulfite, dimethylbutanolamine sulfite, dimethylhexanolamine sulfite and the like; metallic formaldehyde sulfoxylates, such as zinc formaldehyde sulfoxylate, the alkali metal sulfoxylates, such as sodium formaldehyde sulfoxylate and potassium formaldehyde sulfoxylate; alkali metal borohydrides, such as sodium borohydride, potassium borohydride and sodium potassium borohydrate; alkali metal sulfites, such as sodium or potassium bisulfite, sulfite, and metabisulfite; and ammonium bisulfite, sodium sulfide, sodium hydrosulfide; sodium hypophosphite, sodium thiosulfate, sodium dithionate, titanous chloride, sulfuric acid; mercaptan acids, such as thioglycollic acid and its water soluble salts, such as sodium, potassium or ammonium thioglycolate; mercaptans, such as hydrogen sulfide, alkyl mercaptans such as butyl or ethyl mercaptans and mercaptan glycols, such as  $\beta$ -mercapto ethanol; and mixtures of these reducing agents.

Particularly beneficial results are obtained if the reducing agent is employed in conjunction with a "low molecular weight polyhydroxy compound" or other auxiliary agent. Urea constitutes the most readily available and desirable auxiliary agent, although any other material which will swell kertinous fibers in an aqueous medium is suitable. For example, guanidine compounds such as hydrochloride; formamide, N,N-dimethylformamide, acetamide, N,N-dimethylacetamide, thiourea, dimethylsulfoxide, phenol, lithium salts, such as the chloride, bromide, and iodide and the like are similarly useful.

By the term "low molecular weight polyhydroxy compound" is meant a compound containing more than one hydroxy group and having a molecular weight preferably no greater than about 4000. Of these compounds, the most readily available and desirable compound, from the standpoint of ease of application, comprises ethylene glycol. A particularly preferred group of glycols includes the polyfunctional glycols having terminal hydroxyl groups separated by 2 to 10 methylene groups, including, of course, the preferred ethylene glycol as well as trimethylene glycol, tetramethylene glycol, pentamethylene glycol, hexamethylene glycol, and decamethylene glycol, or such glycols as 1,2-propylene glycol, di-propylene glycol, 1,3-butylene glycol, diethylene glycol, polyethylene glycol or the like.

Polyfunctional compounds containing more than 2 hydroxyl groups include the polyfunctional alcohol glycerols such as glycerine and diethylglycerol as well as trimethylol ethane, trimethylol butane, tris-hydroxymethyl-amino methane and others. Glycol ethers, such as the water-soluble or dispersible polyethylene glycols or poly-propylene glycols having molecular weights preferably no greater than about 4000 also provide satisfactory results when utilized in accordance with this invention.

The reducing agent with or without the auxiliary agent or polyhydroxy compound may be applied to the fabric in any desired amount, depending upon the degree of reducing desired. In general, optimum results are obtained when aqueous solutions containing from about 0.01 to about 20% by weight and most preferably from 1 to about 10% by weight of the reducing agent is applied to the fabric. The swelling agent or polyhydroxy compound if employed may be applied to the fabric by addition to the aqueous solution of reducing agent of amounts of from about 3 to about 30% and, most preferably, from about 5 to about 20% by weight. Higher concentrations may be utilized where the fabric is to be exposed to the treating medium for only a short time.

## 11

Subsequent to the external stabilization operation, the fabric may be converted to a garment and the garment subjected to the reducing agent treatment for setting durable configurations in the garment. The conversion to a garment is preferable where the object of the process is to produce creases in the garment which are durable to home laundering. Alternatively, however, the externally stabilized fabric may be impregnated with the desired reducing agent solution, preferably containing a swelling agent or low molecular weight polyhydroxy compound, and then dried under conditions which are not capable of reforming any split linkage in the keratinous fibers. The resulting fabric is thereby presensitized for subsequent durable setting in garment or fabric form on any of the well-known equipment used for setting operations. A particular advantage of such a fabric, with or without a swelling agent and/or low molecular weight polyhydroxy compound, can be made into garments and the garments durably set by standard pressing and curing, for example, using a Hoffman press to impart creases to the garments and then reforming any split linkages in a curing oven. The configurations set in garments in this manner are durable, at the very least, to the wetting, tumbling action of a coin-operated dry cleaning machine. Furthermore, the excellent appearance of such fabrics is substantially retained after wetting.

It is preferred, however, for washability characteristics that water in an amount of at least about 5%, preferably 10 to 40%, or even more, be applied to the presensitized fabrics before pressing and curing.

The mechanical steps of producing a texture effect, crease, and the like may be carried out with any of the well-known existing pieces of textile finishing equipment. For the preparation of creases, however, a Hoffman press is preferred.

The process of this invention is applicable to any keratinous substrate, including, of course, fabrics made from blends of keratinous fibers with other natural fibers, including silk, cellulosic fiber and the like, or with synthetic fibers, such as synthetic cellulosic fibers including acetylated cellulose, for example, the cellulose acetates, acetylated rayon, rayon per se and the like; polyamides, particularly nylon, both 6 and 66 types; polyesters, such as polyethylene terephthalate and the like; polyolefins, such as polyethylene, polypropylene and the like; acrylic fibers such as those produced from acrylonitrile and co-polymers thereof, and the like.

It is preferred, however, that a substantial amount of keratinous fibers, for example, at least about 20%, preferably at least about 40%, by weight be present in the substrates being treated.

The following specific examples of the process of this invention are given for purposes of illustration and should not be considered as limiting the spirit or scope of this invention.

## EXAMPLE I

Into a jacketed stainless steel reactor is poured 225 lbs. of polypropylene glycol adduct of glycerin having a molecular weight of about 5,000. The reactor is then closed and the pressure therein reduced to about 10 mm. mercury after which the reactor is flushed with dry nitrogen. The pressure regulation and flushing operation is repeated for 3 cycles, after which 23 lbs. of dry toluene is poured into the reactor. A blanket of nitrogen gas is maintained in the vessel throughout the reaction. The pressure is again reduced to 10 mm. mercury and the reactor is heated to 140° C. to distill off the toluene, after which it is cooled to room temperature using cold water in the jacket around the reactor. The pressure is returned to room conditions. After stirring for 15 minutes to thoroughly mix the components about twice the stoichiometric quantities for reaction with the glycol of toluylene - 2,4 - diisocyanate is added rapidly and stirred until the heat of reaction ceases and the temperature has

## 12

risen slowly up to 40-45° C. from room temperature of about 28° C. The reaction mix is then heated at a rate of about 2° C. per minute to a temperature of 146° C. where it is held for 18 minutes and then cooled at a rate of about 2° C. per minute to a maximum temperature of 100° F. Sufficient trichloroethylene is then added to provide a solution containing 70% of the resulting prepolymer. The pre-polymer solution is then transferred from the reactor to a pre-dried drum under a dry nitrogen atmosphere to avoid water contamination. At the time of the transfer, the pre-polymer solution has a color of from colorless to a very pale straw color.

A solution is then prepared from the 70% solution of the prepolymer by dilution with additional trichloroethylene, the dilution being conducted to the point so that a pickup of 3.5% based on the dry weight of the fabric of prepolymer is picked up on the fabric. N,N, N'N'-tetrakis 2-hydroxy propyl ethylene diamine in the amount of about 3% of the weight of pure prepolymer is added to the bath. The solution is padded onto the wool fabric and the padded fabric is then placed in an oven at 160° F. for 5 minutes for drying and then placed in the second oven at 250° F. for 5 minutes for curing. The treated fabric is then scoured, dried and pressed. Trousers are then prepared from the urethane treated fabric. The trousers are sprayed with a 6.4% solution of monoisopropynolamine sulfite to a wet pickup of 40%, allowed to stand in the damp state for one hour and then creases are pressed in the trousers by means of a Hoffman press employing a 30 second top stream, a 30 second bake and a ten second vacuum. The creases and dimensional stability of the trousers are found to be durable to several washing cycles in a Kenmore washer, employing commercially available detergents, e.g., Tide brand detergent, in recommended quantities, and employing tumble drying cycles after each wash cycle. The creases and dimensional stability of the trousers are also durable to multiple dry cleaning operations.

## EXAMPLE II

The procedure of Example I is repeated with the exception that in place of the 70% solution of the prepolymer employed in Example I to effect the external stabilization, a "one-shot" polyurethane external stabilization technique is employed. The "one-shot" polyurethane solution is prepared as follows: Sufficient amount of the polypropylene glycol adduct of glycerine employed in Example I to prepare the prepolymer is added to the trichloroethylene pad bath so that pickup of 2.5% based on the dry weight of the fabric of polypropylene glycol adduct is effected. Sufficient methylene-di-p-phenyl diisocyanate is added so that a pickup of 0.5% based on the dry weight of the fabric of the diisocyanate is effected. A quantity of 8% zinc naphthenate solution is added amounting to 3% of the weight of polypropylene glycol adduct and employed diisocyanate. The solution is padded onto the fabric and process thereafter carried out substantially as set forth in Example I. The finished product is found to have a crease and dimensional stability which is durable to several washing cycles employing commercially available detergents, e.g., Tide brand detergent, in recommended quantities, and employing tumble drying cycles after each wash cycle.

## EXAMPLE III

The procedure of Example II is repeated with the exception that the fabric upon being formulated into a pair of trousers is sprayed instead with an aqueous solution containing 2% by weight sodium bisulfite, 5% urea and 0.2% Decersol OT.

## EXAMPLE IV

An all wool worsted flannel fabric is given the external stabilization treatment as set forth in Example I. The

open width externally stabilized fabric is then padded with a solution containing 3% by weight sodium bisulfite and 0.2% by weight Deceresol OT. Alternatively, a solution containing 3% by weight sodium bisulfite, 5% by weight urea, and 0.2% by weight Deceresol OT may be employed. The treated fabric is dried at 175° F. and given a light press. The fabric is then fashioned into two pairs of trousers. One pair of trousers is sprayed with water containing 0.2% Deceresol OT to a pickup of about 40% by weight based on the dry weight of the fabric. After standing in the damp state for 30 to 60 minutes creases are pressed into the trousers by means of a Hoffman press, using a cycle of 30 seconds top steam, 30 seconds bake, 10 seconds vacuum, at a steam pressure of 80 p.s.i. The trousers are then dried for 15 minutes in an oven at a temperature of 325° F. The crease and dimensional stability of the fabric is found to be durable to several washing cycles in a Kenmore washer, employing commercially available detergents, e.g., Tide brand detergent, in recommended quantities, and employing tumble drying cycles after each wash cycle.

The other pair of trousers is similarly pressed and heated in the oven but without prior wetting with water. The creases so imparted are durable to the effects of a coin-operated dry cleaning unit, but do not withstand the washing operations as well as the other pair of trousers which were wetted before pressing. Similar, though slightly improved, results are obtained when ethylene glycol is substituted for urea and the above procedures are repeated.

#### EXAMPLE V

The procedure as set forth in Example IV is repeated with the exception that the fabric is stabilized externally according to the procedure set forth in Example II.

#### EXAMPLE VI

The procedure set forth in Example IV is repeated with the exception that the externally stabilized fabric is padded with a solution containing 3% by weight sodium bisulfite, 5% urea and 0.2% Deceresol OT.

#### EXAMPLE VII

The polyurethane external stabilization process set forth in Example I was again repeated and the externally stabilized fabric again subjected to a scouring, drying and finally a pressing operation. The stabilized fabric is then converted into trousers and the trousers sprayed with an aqueous solution containing 2% by weight sodium bisulfite and 0.2% by weight Deceresol OT (synthetic surfactant agent marketed by American Cyanamid Company) and 5% by weight urea. The spraying is conducted in a fashion so as to produce a pickup of about 40% by weight based on the dry weight of the fabric. The sprayed trouser is then pressed in a Hoffman press. The crease and dimensional stability of the final product is found to be durable to several washing cycles in a Kenmore washer, employing commercially available detergents, e.g., Tide brand detergent, in recommended quantities, and employing tumble drying cycles after each wash cycle.

#### EXAMPLE VIII

An all wool worsted flannel is solvent dry cleaned and is dried free of solvent. The cleaned fabric is then dipped into an emulsion prepared as follows: (a) 4 grams of the polyester reaction product of adipic acid and glycerol is dissolved in 4 milliliters of methylethyl ketone (b) 4 grams of 2,2 bis(2,3-epoxy-propoxy phenyl) propane was dissolved in 4 milliliters of methylethyl ketone (c) 4 grams of polyamide condensation product of diethylene triamine and dimerized unsaturated fatty acid was dissolved in 4 milliliters of methylether ketone. The 3 solutions of (a), (b), and (c) are then mixed together and the composite solution poured into 375 milliliters of water with stirring so as to form an emulsion. The dry cleaned

cloth is then dipped into the emulsion and passed through squeeze rolls so as to give a weight increase of 65%. The impregnated fabric is air dried to about 30% moisture and then heated in an oven for 30 minutes at 250° F. A pair of trousers is then prepared from the externally dimensionally stabilized fabric. The trousers are then sprayed with a 6.4% solution of N-propanolamine sulfite to a wet pickup of about 50%. The trousers are then allowed to stand for one hour in the damp state and then creases are pressed in the trousers by means of a Hoffman press employing a 30 second top steam, a 30 second bake and a 10 second vacuum. The trousers are found to have dimensional stability and crease stability after several washing cycles in a Kenmore washer, employing commercially available detergents, e.g., Tide brand detergent, in recommended quantities, and employing tumble drying cycles after each wash cycle.

#### EXAMPLE IX

20 The external stabilization process set forth in Example II was again repeated and the externally stabilized fabric formed into a pair of trousers. The trousers are then sprayed with an aqueous solution containing 2% by weight sodium bisulfite and 0.2% by weight Deceresol OT. The remainder of the processing operations were conducted substantially in accordance with the process set forth in Example II. The final product was found to have dimensional stability and crease stability after several home laundering cycles in a Kenmore washer, employing commercially available detergents, e.g., Tide brand detergent, in recommended quantities, and employing tumble drying cycles after each wash cycle.

#### EXAMPLE X

35 A 50% polyester, 50% wool worsted flannel fabric is immersed in a 3.3% aqueous solution of polyamino-caproic acid, diethyl amino ethanol derivative, the specific means of preparation of which is set forth in U.S. Patent No. 2,696,448. Excess pad liquor is removed by passing the fabric through squeeze rollers. The fabric is dried at about 80° C. and then cured at 130° C. for 15 minutes. The externally stabilized fabric is then treated with the reducing agent solution substantially as set forth in Example I. The finished product is found to have dimensional stability and crease stability even after being subjected to several washing cycles in a Kenmore washer, employing commercially available detergents, e.g., Tide brand detergent, in recommended quantities, and employing tumble 45 drying cycles after each wash cycle. The finished product is also found to have dimensional stability and crease stability to multiple dry cleaning operations.

#### EXAMPLE XI

55 The procedure of Example V is repeated with the exception that subsequent to the external stabilization operation, the fabric upon being formulated into a pair of trousers is sprayed with an aqueous solution containing 2% by weight sodium bisulfite and 0.2% by weight Deceresol OT, the remaining treatment being conducted substantially as set forth in Example V. The finished product is found to have dimensional and crease stability after having been subjected to several home laundering operations which include the use of commercially available detergents and tumble drying operations.

Having thus disclosed the invention, what is claimed is:

1. A process for durably setting a fabric containing keratinous fibers in a desired configuration comprising (a) treating said fabric with a monomeric polyisocyanate and a polymeric polyfunctional compound selected from the class consisting of polymeric polyhydroxy compounds, polyesters, polyamides, polyepoxides and reaction products of phenol and alkanol oxides, formaldehyde resins, hydrogenation products

15

- of olefin-carbon monoxide copolymers and polyepi-halohydrins,  
 (b) curing said treated fabric to externally stabilize the fabric,  
 (c) treating the stabilized fabric with a reducing agent,  
 (d) maintaining the reducing agent treated fabric in a desired configuration, and  
 (e) heating the fabric to a temperature sufficient to set the fabric in the desired configuration.  
 2. The process of claim 1 wherein the fabric is an all wool fabric.  
 3. The process of claim 1 wherein the polymeric poly-functional compound is a polyether polyol.  
 4. The process of claim 1 wherein the isocyanate is an aryl diisocyanate.  
 5. The process of claim 1 wherein the isocyanate is a blocked isocyanate which is activated by heating at an elevated temperature.  
 6. The product of the process of claim 1.

16

## References Cited

## UNITED STATES PATENTS

|           |        |               |       |           |
|-----------|--------|---------------|-------|-----------|
| 3,098,694 | 7/1963 | Reider        | ----- | 8—128     |
| 2,710,816 | 6/1955 | Evans et al.  | ----- | 8—128     |
| 3,078,138 | 2/1963 | Miller et al. | ----- | 8—127.6 X |

## FOREIGN PATENTS

|         |        |               |       |         |
|---------|--------|---------------|-------|---------|
| 968,534 | 9/1964 | Great Britain | ----- | 8—127.6 |
|---------|--------|---------------|-------|---------|

DONALD LEVY, Primary Examiner

J. CANNON, Assistant Examiner

## U.C. CL. X.R.

15 8—115.5, 115.7, 127.5, 128 A, 128 R, 129, DIG. 4;  
 38—144; 2—243; 8—DIG. 9, DIG. 11, DIG. 21;  
 117—141, DIG. 7